

# UNITED STATES PATENT OFFICE.

MARK W. MARSDEN, OF PHILADELPHIA, PENNSYLVANIA.

## OBTURATING MATERIAL.

1,192,662.

Specification of Letters Patent. Patented July 25, 1916.

No Drawing.

Application filed December 13, 1915. Serial No. 66,512.

*To all whom it may concern:*

Be it known that I, MARK W. MARSDEN, a citizen of the United States, residing at Philadelphia, in the county of Philadelphia and State of Pennsylvania, have invented 5 certain new and useful Improvements in Obturating Material, of which the following is a specification.

One of the principal objects is to provide 10 a comparatively inexpensive, highly efficient and exceedingly durable material or means for obturating purposes, mainly intended for marine use and particularly in connection with armored craft to prevent flooding 15 in the event the hull is breached or ruptured either from internal or external causes.

Another object is to provide a material of 20 the character stated, which may not be fired by spark or flame, the friction of penetrating projectiles, or from any cause whatsoever.

Another object is to provide a material of 25 the character stated, which is immune to dry-rot and is not deleteriously affected by sweating moisture or by changing temperatures or by age and will not generate poisonous gases.

Another object is to provide a highly absorptive, yielding and resilient material 30 adapted instantly to close a breach resulting from the impact of a projectile or from other cause.

Another object is to provide an obturating 35 material, which, while comparatively light, will, upon functioning, have no tendency to wash away.

Otherwise stated, the purpose of the present invention is to overcome the defects and disadvantages of the obturating materials 40 heretofore proposed.

In practising the invention I use a product composed essentially of mineral fiber and a very light material having springy or expansive properties and designed to 45 prevent the mineral fiber from overcompacting. Cork in granular or comminuted state answers the requirements, the other components being mineral wool and asbestos. The product consists of the combination of these 50 elements in loose as distinguished from sheet or fabricated form. Before combining these elements I first subject the cork in a granu-

lated or comminuted state to a fireproofing process. The latter may be any of the approved methods, but I prefer to use a hot 55 chemical solution, preferably alum and sal ammoniac and hot water. The cork is then thoroughly dried and associated with the mineral fiber in the ratio of twenty per cent., more or less, mineral wool and ten per cent., 60 more or less, asbestos. In some cases more mineral fiber is desirable. As before stated the mineral fiber is in loose or flocky form and the mixing is performed in such way as to uniformly distribute the components. 65 The product of the mixture is then compressed to a density of from twelve to twenty pounds per cubic foot. The presence of the cork makes for lightness and resiliency and for a product having absorptive 70 properties in excess of any heretofore proposed. This is because the cork particles operate as yielding or resilient separating elements, which prevent the fibers from compacting too much, and hence enable the 75 product to swell or expand rapidly under the influence of water and to retain or take care of a larger bulk of water than was heretofore possible. The fibers readily interlace and mat with one another and with the cork 80 and prevent the latter from washing away.

Having described the nature and objects of the invention, I claim:—

1. Obturating material consisting of a compressed product of mineral fiber and an 85 element adapted and arranged to prevent undue compacting.

2. Obturating material consisting of a compressed product of mineral wool and asbestos and an element adapted and arranged 90 to prevent undue compacting.

3. Obturating material consisting of a mixture of mineral wool and asbestos and springy separating elements scattered 95 throughout the same.

4. Obturating material consisting of a mineral wool and asbestos combined in loose or flocky form with a light, buoyant, flexible, fireproofed material.

5. Obturating material consisting of a 100 dense or compressed product of a mixture in loose form of granular cork and mineral fiber.

6. Obturating material consisting of a

dense or compressed product of granular cork initially treated to make it fireproof and mineral fiber.

7. Obturating material consisting of a dense or compressed product of granular cork, initially treated to make it fireproof, mineral wool and flocky asbestos.

In testimony whereof I affix my signature in the presence of two witnesses.

MARK W. MARDEN.

Witnesses:

ALLAN I. HUCKINS,  
E. W. STRAIN.